

## UNITED STATES PATENT OFFICE

2,580,491

REDUCING THE CRYSTALLINITY OF NATIVE  
FIBROUS CELLULOSIC MATERIAL

Kyle Ward, Jr., and Carl M. Conrad, New Orleans,  
and Leon Segal, Metairie, La., assignors to the  
United States of America as represented by the  
Secretary of Agriculture

No Drawing. Application August 8, 1950,  
Serial No. 178,339

10 Claims. (Cl. 260—212)

(Granted under the act of March 3, 1883, as  
amended April 30, 1928; 370 O. G. 757)

1

The invention herein described may be manufactured and used by or for the Government of the United States of America for governmental purposes throughout the world, without the payment to us of any royalty thereon.

This invention relates to native fibrous cellulosic material, in particular cotton, linen, ramie, and other vegetable fibrous materials, in which the crystal form of cellulose I (native cellulose), as well as the fibrous structure, of the original native material is retained but in which the degree of crystallinity is reduced.

The objects of the present invention are, first, to provide a fibrous cellulosic material, such as cotton, in which the original high degree of crystallinity of 85–90% has been reduced to varying and controllable degrees down to as low as about 20%, and where such reduction has been retained to a greater or less degree after completion of the treatments necessary to accomplish the reduction; second, to prepare this cellulosic material of low crystallinity in a manner such that there is substantially no chemical degradation and substantially no loss or impairment of the fibrous structure; and third, to prepare this cellulosic material of low crystallinity without changing the crystal form from that of cellulose I (native cellulose).

For an understanding of the present invention, an exposition of the present view of cellulose, as it occurs in nature, especially in the vegetable fibers, is pertinent. Such cellulose is considered to be composed of two modifications, or phases. One of these is the dense crystalline phase, giving rise to characteristic X-ray diffraction patterns, and believed to consist of minute fibrous crystals, composed of many parallel cellulose molecules, lying side by side, and held together in exact relation by forces known as hydrogen bonds. The crystals are not, in fact, discrete, but are considered to be connected by long cellulose molecules which, in proceeding from one end of the molecule to the other, may pass through a dozen or more crystallites and intercrystalline regions. There is produced, thus, a discontinuous crystalline structure, held together by the interconnecting, but widely diverging, cellulose chains. The intercrystalline portions of the cellulose molecules constitute a continuous network, and thus represent the less dense, so-called, amorphous modification or phase. Unlike the crystalline fraction, this latter phase gives rise to a broad halo when irradiated in the X-ray beam.

One of the principal drawbacks of the native

cellulosic fibers is their brittleness and tendency to fail when subjected to combined strain and shock. Thus, in spite of the great strength of such cellulosic fibers as flax and ramie, they have never attained much use in automobile tires and other mechanical fabrics due to their inability to resist shock. This shortcoming is considered to be associated with the high degree of crystallinity of these fibers, being in the range of 90–95%. Cotton fibers do not show the degree of failure from shock that is shown by the flax, ramie, and other bast fibers generally, and this is believed to be due to the somewhat lower crystallinity of cotton fibers, which vary from 85–90%. However, it is considered that the crystallinity of cotton fiber, notwithstanding its somewhat lower value, is nevertheless considerably greater than optimum, and that a material improvement would be accomplished by the production of a fiber otherwise the same, but lower in crystallinity.

The crystallinity of cotton fiber, and native cellulosic fibers generally, militates against their maximum usefulness in still another way. The fibers are dense and rather impervious to gases, liquids, reagents, etc. This is manifest in a number of ways. Cotton fibers, together with cellulosic fibers in general, as is well known, are rather poorly sensitive to dyeing, and must be dyed with certain substantive dyes, i. e., dyes that will adsorb on cellulose, or with mordant dyes. It is believed that the relatively large dye molecules cannot penetrate the crystalline areas, but only the relatively large areas, crevices, and pores existing in the amorphous areas. Many types of dye molecules being relatively small can pass into the amorphous areas, but due to the open structure, can pass out readily and are not retained on removal of the dye bath and washing. Since the amorphous areas can thus be considered to be the active adsorbing center of the fiber, it follows that any process which provides an increase of amorphous component at the expense of the crystalline component will greatly increase and improve the dye-absorbing capacity of cellulose, permitting more economical application, and more brilliant products to be formed.

The dense and unsatisfactory nature of native fibrous cellulose is disclosed again when it is reacted in the fibrous condition with such reagents as acetyl, propionyl, butyryl and benzoyl anhydrides; methyl, ethyl, and propionyl alcohols; and numerous other substances. For example, the acetylation reaction, as is well-known, takes place very rapidly up to an extent corresponding

approximately to the amount of amorphous cellulose present, and then much more slowly throughout the remainder of the reaction. The interpretation is that the reaction occurs principally in the amorphous areas and perhaps on the surfaces of the crystallites. If the cellulose were first transformed into a product with a high proportion of amorphous cellulose, it is considered that the rate of reaction could be greatly accelerated and the cost of manufacture correspondingly reduced.

It is considered, in fact, that all reactions with fibrous cellulose must take place in two ways; first, very rapidly in the accessible, exposed, regions, i. e., in the amorphous areas; and secondly on the surfaces of the crystallites, by a much slower "topochemical" reaction. The surfaces of the crystallites being necessarily small in comparison with the surfaces exposed by the amorphous regions, it follows that the relative proportion of the latter must be the predominant factor in determining ease and rate of reaction. Any process which generates amorphous cellulose at the expense of the crystalline fraction must facilitate and favor the desired reaction.

In general according to the present invention, the native fibrous cellulosic material, particularly cotton, is treated by immersion in an anhydrous, liquid primary alkyl amine containing 1 or 2 carbon atoms preferably primary ethylamine, or in a mixture of such amines and an anhydrous primary alkyl amine containing 6 or 7 carbon atoms, preferably primary hexylamine. A substantial amount of the treating agent is then mechanically removed from the treated material, substantially all of the remaining agent being removed by extraction with a non-polar solvent, such as chloroform. This produces a fibrous cellulosic material with crystallinity ranging from about 20% to about 50%, according to the conditions of treatment. Reduction of crystallinity varies with the time of immersion in the amine, periods of from 4-16 hours resulting in the lowest crystallinity. The physical condition of the fiber during treatment is such that handling is not difficult. There are no visible signs of fiber damage, which fact is verified by the results of accepted tests on the material.

X-ray diffraction patterns of such treated celluloses are those of cellulose I, but the heights of the characteristic diffraction peaks are much reduced, indicating reduced crystallinities in qualitative agreement with the results of the principal crystallinity determinations used.

Determinations of the change in the crystallite size in the treated celluloses show that this decreases from about 210 glucose units for the untreated cotton to about 110 glucose units for the treated cotton.

Immersion of the treated cellulose in boiling water for as long as 3 hours causes only a partial restoration of crystallinity provided it has been reduced below that 50%, and with no change in the type of crystal form. Regardless of how low the reduced crystallinity may have been carried originally, after boiling in water it is found to be in the range of 50-60%.

The treated cellulose exhibits an increased moisture regain as well as increased water retention or imbibition. Increases in these parameters are accepted as indicative of increased amorphous material, i. e., of reduced crystallinity.

The results of accepted tensile tests made on yarns and cords show that, first, the breaking strength has not been significantly changed by

the treatment; second, the percent elongation-at-break has been more than doubled thus resulting in nearly doubling the toughness. These effects are in agreement with the concept of reduced crystallinity. Determination of twist by an accepted method shows that there has been no significant change in the twist of the yarn by the treatment.

Higher alkyl amines, such as normal hexylamine, even though anhydrous when used alone as the treating agent, do not reduce crystallinity. However, these higher amines, particularly primary hexyl- and primary heptylamines, when preceded by a short-chain amine, particularly anhydrous liquid ethylamine, can effect a further reduction in the crystallinity which has already been reduced by the short-chain amine; but this additional reduction amounts only to about 5%. If the long- and short-chain amines are mixed together, proportions of 75% short-chain amine, particularly ethylamine, and 25% long-chain amine, particularly hexylamine, by weight, must be used to obtain crystallinities of about 50%. Varying the proportions will affect the amount of reduction. Thus, no reduction is found if the amines are in the proportions where the short-chain amine is present as 50% or less, by weight.

Since the short-chain amines have low boiling points and since a continuous cyclic method of extraction is employed to remove from the swollen cellulosic material such amine as remains after washing with the non-polar solvent, a means must be provided to prevent them from cycling with the solvent. A suitable method of doing this was to form in the boiling flask of the extractor a non-volatile amine salt which may or may not be soluble in the solvent. Aqueous solutions of acidic material are unsuitable since the presence of water is to be avoided; volatile acidic substances are to be avoided for reasons obvious to those skilled in the art; whatever the substance, or substances, there must not be an adverse reaction with the solvent. Concentrated orthophosphoric acid plus a small amount of phosphoric anhydride was found to be suited for this purpose. Sulfamic acid can serve the purpose also, but concentrated sulfuric acid is not suitable since it reacts adversely with the solvents.

The following examples, which are not to be considered as limiting, illustrate the process of treating the cellulosic fiber.

#### Example I

Approximately 10 g. of bleached cotton fiber, obtained from a commercial source and cut to short lengths, was immersed overnight at 5° C. in anhydrous liquid monoethylamine, contained in a screw-cap bottle. No attempt was made to exclude air during the handling or processing. After preliminary removal of the amine by suction, followed by washing and extracting of the remainder with chloroform, the cotton was allowed to dry. The crystallinity of this material was found to be about 23%. It was still fibrous and visually apparently undamaged; however, by viscosity measurements it was found to show some chemical degradation which was attributed to alkaline oxidation due to exposure to atmospheric oxygen.

#### Example II

About 100 g. of the cut cotton described in Example I was immersed for 4 hours in anhydrous, liquid monoethylamine at 0° C. contained in a vessel open to the atmosphere. Excess amine

was removed by suction. The cotton, still damp with ethylamine, was placed in a large screw-cap bottle and then covered with anhydrous normal hexylamine. The bottle and contents were allowed to stand overnight at room temperature. The excess hexylamine was removed by suction, then by washing and extracting with chloroform. No attempts were made to exclude air during the handling and processing. After drying, this material was found to have a crystallinity of about 19%, and was still fibrous and apparently undamaged.

*Example III*

Approximately 10 g. of cut cotton as described in Example I was immersed overnight at room temperature in a mixture of amines. The mixture consisted of 75% by weight of anhydrous monoethylamine and 25% by weight of anhydrous normal hexylamine. The cotton and amine mixture was contained in a closed glass jar of sufficient strength to withstand considerable internal pressure. By morning some pressure had developed, evidently from the high content of ethylamine in the mixture, but this was easily vented before attempting to open the jar. The liquid was removed by suction, followed by washing and extracting with chloroform. After drying, the fibrous material was found to have a crystallinity of 50%.

*Example IV*

Approximately 10 g. of cut cotton, as in Example I, was treated exactly as given in Example I, with the exception that normal hexane was used instead of chloroform for washing and extracting the treated material. After air-drying, the crystallinity of the fibrous material was found to be about 20%.

*Example V*

Four approximately 10 g. samples of the cut cotton described in Example I were each immersed for different lengths of time in anhydrous monoethylamine. These times were 5 and 30 minutes, 2 and 4 hours, and the crystallinities after removal of the amine, as described in the above examples, were 44, 42, 32, and 24%, respectively.

*Example VI*

One pound of raw cotton fiber, in the form of card sliver, was treated with anhydrous ethylamine. Batches of 100 g. each of the sliver, in continuous form, were immersed 4 hours in the anhydrous amine. All operations were carried out under nitrogen, including the first two washings with chloroform to begin removal of the amine. The remainder of the amine was removed by extraction with chloroform. After air-drying, the fiber was found to have a crystallinity of 24%. Critical examination of the fiber revealed that there was very little degradation. The sliver had a harsh hand, due to the removal of the waxes by the treatment.

*Example VII*

The exact treatment as described in Example VI above was repeated on 10 g. skeins of a 20's singles, kier-boiled cotton yarn of loose twist.

After drying, the yarn, of undamaged appearance and slightly harsh hand, had a crystallinity of 31%.

*Example VIII*

The exact treatment described in Example VI above was repeated on 10 g. skeins of the 20's singles yarn. In this case the crystallinity of the extracted, dry yarn was 34%. There was little degradation and only a slightly harsh hand. The yarn was still suitable textile material as evidenced by tensile tests for breaking strength and elongation.

Having described our invention, we claim:

1. A process of reducing the degree of crystallinity of a native fibrous cellulosic material with no substantial chemical degradation and impairment of the fibrous structure comprising immersing the cellulosic material in a liquid treating agent selected from the group consisting of an anhydrous primary alkylamine containing from 1 to 2 carbon atoms, and a mixture of at least 50% by weight of an anhydrous primary alkylamine containing from 1 to 2 carbon atoms and an anhydrous primary alkylamine containing from 6 to 7 carbon atoms, mechanically separating a substantial amount of the treating agent from the treated material, and separating substantially all of the remaining treating agent by extraction with a non-polar organic solvent.
2. The process of claim 1 in which the treating agent is anhydrous primary methylamine.
3. The process of claim 1 in which the treating agent is anhydrous primary ethylamine.
4. The process of claim 1 in which the treating agent is a mixture of at least 50% by weight of an anhydrous primary alkylamine containing from 1 to 2 carbon atoms and an anhydrous primary alkylamine containing from 6 to 7 carbon atoms.
5. The process of claim 1 in which the treating agent is a mixture of at least 50% by weight of anhydrous primary ethylamine and anhydrous primary hexylamine.
6. The process of claim 1 in which the non-polar solvent is chloroform.
7. The process of claim 2 in which the non-polar solvent is chloroform.
8. The process of claim 3 in which the non-polar solvent is chloroform.
9. The process of claim 4 in which the non-polar solvent is chloroform.
10. The process of claim 5 in which the non-polar solvent is chloroform.

KYLE WARD, JR.  
CARL M. CONRAD.  
LEON SEGAL.

**REFERENCES CITED**

- 60 The following references are of record in the file of this patent:

**UNITED STATES PATENTS**

| Number    | Name              | Date          |
|-----------|-------------------|---------------|
| 2,186,101 | Dreyfus           | Jan. 9, 1940  |
| 2,200,452 | Kosslinger et al. | May 14, 1940  |
| 2,218,479 | Peterson          | Oct. 15, 1940 |
| 2,270,326 | Miller            | Jan. 20, 1942 |